

## UNITED STATES PATENT OFFICE

2,449,768

HEAT-TREATING MAGNESIUM-ALLOY  
DIE CASTINGS

Robert C. Cornell, Jackson, Mich., assignor to The Dow Chemical Company, Midland, Mich., a corporation of Delaware

No Drawing. Application August 1, 1946,  
Serial No. 687,703

4 Claims. (Cl. 148—21.90)

1

This invention relates to the heat-treatment of magnesium-base alloy pressure die-castings.

Magnesium-alloy sand and permanent-mold castings are conventionally heat-treated to develop improved properties. However, the application of similar heat-treatment to pressure die-castings of the same metal has been largely unsuccessful. Thus, while such die-castings are sometimes given a conventional solution-heat-treatment to relieve stresses or to improve ductility, there has always been an accompanying serious decrease in yield strength. Aging treatments likewise decrease the strength of the casting and also lower the ductility. For these reasons, magnesium-base alloy die-castings have almost always been used in the as-cast condition.

It has now been found, however, that both the strength and the ductility of magnesium-base alloy die-castings may be materially improved by solution-heat-treatment, provided the castings are first subjected to artificial aging. This discovery forms the basis of the present invention.

In practice of the invention, the pressure die-cast article of a solution-heat-treatable magnesium-base alloy, in the as-cast condition, is first heated at an aging temperature for a time sufficient to produce substantial precipitation of a major additional phase in the alloy. In the case of the common magnesium die-casting alloys containing from 4 to 12 per cent by weight of aluminum as the major alloying element, temperatures in the range of 325° to 700° F. are preferred, with times of at least several hours being usually required. For example, a magnesium-base alloy containing 8 to 10 per cent of aluminum, 0.4 to 1.0 per cent zinc, and 0.1 to 0.5 per cent manganese as the major alloying elements is best aged at from about 325° to about 550° F. for a period of from about 5 to about 20 hours, the longer times being required at the lower temperatures.

Following the aging procedure, the article is then given a solution-heat-treatment for a time sufficient to effect a partial or preferably a nearly complete solution of the precipitated additional phase. Temperatures conventional for solution-heat-treating magnesium-alloys are employed, the times of heating being slightly less than those ordinarily used with sand-cast magnesium articles. For example, with the 4 to 12 per cent aluminum-containing alloy, a temperature of at least 715° F. for at least several minutes is preferred. In the case of the magnesium-aluminum-zinc-manganese alloy mentioned above, the solution-heat-treatment is best carried out at from

2

760° to 790° F. from a time of from about 15 minutes to about 2 hours.

Following the solution-heat-treatment, the article is cooled to room temperature and is ready for use.

Metallographic studies give a possible explanation of the effectiveness of the heat-treatment according to the invention. Thus, when die-cast magnesium alloy articles are subjected to solution-heat-treatment without preliminary aging, a non-germinative but regular grain growth occurs, with resultant weakening of the metal. However, when the die-cast article is first given a precipitation or aging heat-treatment according to the invention and is then solution-heat-treated, grain growth during the latter treatment is minimized or even inhibited and the strength and ductility of the metal are improved. This inhibiting effect persists throughout solution-heat-treatment, even well after the phase precipitated during the aging has been dissolved. The precise cause of the inhibitory effect induced by the aging is not clear but presumably involves some changes in the energy relations in the crystal lattice of the metal. The effect is limited to pressure-die-cast articles in which a high degree of supersaturation exists due to the drastic chilling of the metal, and is not observed in sand and permanent-mold castings of the same magnesium-base alloys.

Since unsound die-castings of magnesium-alloys tend to blister during heat-treatment, it is important, in practicing the invention, to control the initial die-casting operation, in known manner, to produce only sound metal.

The following example will illustrate the invention.

*Example*

40 A magnesium-base alloy containing 9.0 per cent by weight of aluminum, 0.6 per cent zinc, and 0.2 per cent manganese as the major alloying elements was pressure-die-cast into test bars in a standard cold-chamber casting machine. In the as-cast condition, the metal exhibited the following properties: tensile strength, 35,000 p. s. i., yield strength, 22,000 p. s. i., and elongation in 2 inches, 4.0 per cent.

45 The test bars were then subjected to an aging treatment at 500° F. for 18 hours, after which they were given a solution-heat-treatment at 780° for 1.0 hour. The metal then had the properties: tensile strength, 38,000 p. s. i., yield strength, 18,000 p. s. i., and elongation in 2 inches, 10 per cent.

What is claimed is:

1. A heat-treatment for pressure die-cast articles formed of a solution-heat-treatable magnesium-base alloy which consists in heating the as-cast article at an aging temperature for a time sufficient to effect substantial precipitation, and then subjecting the article to solution-heat-treatment.

2. A heat-treatment for pressure die-cast articles formed of a solution-heat-treatable magnesium-base alloy containing from 4 to 12 per cent by weight of aluminum as the major alloying element which consists in heating the as-cast article at an aging temperature in the range of 325° to 700° F. for a time sufficient to effect substantial precipitation, and then subjecting the article to solution-heat-treatment at a temperature of at least 715° F.

3. A heat-treatment for pressure die-cast articles formed of a magnesium-base alloy containing 8 to 10 per cent by weight of aluminum, 0.4 to 1.0 per cent zinc, and 0.1 to 0.5 per cent manganese as the major alloying elements which consists in heating the as-cast article at an aging temperature of from about 325° to about 550° F. for a period of from about 5 to about 20 hours to

effect substantial precipitation, and then subjecting the article to a solution-heat-treatment at a temperature of from about 760° to 790° F. for a time of from about 15 minutes to about 2 hours.

5 4. In a process wherein a pressure die-cast article formed of a solution-heat-treatable magnesium-base alloy is to be solution-heat-treated, a pre-treatment for minimizing grain growth during the solution-heat-treatment which comprises heating the article in the as-cast condition at an aging temperature for a time sufficient to effect substantial precipitation.

ROBERT C. CORNELL.

#### 15 REFERENCES CITED

The following references are of record in the file of this patent:

#### UNITED STATES PATENTS

20 Number Name Date  
2,363,394 Busk Nov. 21, 1944

#### OTHER REFERENCES

Transactions A. I. M. E., vol. 161, page 311.  
25 Published in 1945 by the Institute of Mining and Metallurgical Engineers, New York, New York.